

# UNITED STATES PATENT OFFICE.

FRED R. REED, OF HIGHLAND PARK, MICHIGAN.

## CARBON-REMOVER.

1,227,667.

Specification of Letters Patent. Patented May 29, 1917.

No Drawing.

Application filed March 18, 1916. Serial No. 85,049.

To all whom it may concern:

Be it known that I, FRED R. REED, a citizen of the United States of America, residing at Highland Park, in the county of Wayne and State of Michigan, have invented certain new and useful Improvements in Carbon-Removers, of which the following is a specification.

This invention relates to compounds for removing carbon and more particularly to a compound adapted for removing the carbon from the cylinders of internal combustion engines.

Among the objects of the invention are to provide a carbon remover which when inserted in the cylinders and heated up will commence to immediately disintegrate the carbon deposits, and will continue to act thereon for a considerable period of time, thus causing the carbon deposits to be removed in finely divided particles; to provide a carbon remover which can be economically manufactured and put up in convenient form to be sold to the trade; to provide a carbon remover which automobile users can, without special skill or training, safely and effectively employ for removing the carbon from their engines; and in general to provide a new and improved compound of the character above referred to.

In the ordinary use of internal combustion engines there is a coating or crust of carbon deposit formed on the interior surface of the cylinder and on the piston, valves and other interior parts of the engine. Owing to the inaccessibility of these parts it is difficult to mechanically remove the carbon without completely dismantling the engine. The present invention contemplates an improved compound, which can be easily inserted in the cylinders and by which this carbon deposit can be disintegrated into a finely divided or powdered form, the operation of removing the carbon being accomplished without any injurious effect to the working parts of the engine.

I have found that a compound containing the following ingredients in substantially the following proportions is well

adapted for this purpose. This compound 50 includes:

|                                       |     |
|---------------------------------------|-----|
| Powdered zinc -----                   | 60% |
| Paraffin wax -----                    | 25% |
| Stearin -----                         | 10% |
| Naphthalene (with coloring matter) -- | 5%  |

In its broader aspects the invention is of course not limited to the particular substances and proportions stated, for instance camphene could be substituted for the naphthalene where the cost of camphene would permit of such substitution. While in the preferred form both stearin and naphthalene are employed, the invention in certain of its aspects is not limited to the use of either 65 or both of these substances. Also the proportions of zinc could be varied from a maximum of about 70% down to a minimum of about 30%. However I preferably employ the zinc in substantially as large a percentage as the base will carry. In the above compound the zinc and naphthalene are the active agents while the wax forms the body or base for carrying the active agents and the stearin serves to further hold the zinc 70 in suspension. In commercial use the compound is preferably made up into tablets of suitable size, such as a tablet five-eighths of an inch in diameter by three-eighths of an inch in thickness and the manner of 75 using the compound is as follows:

The motor is started and warmed up. It is then stopped and the spark plugs removed and one or two tablets of the carbon remover inserted into the cylinder. The 85 spark plugs are replaced into position, the motor is started slowly and allowed to run idle for two or three minutes, enough to melt the wax base after which the motor is ready to use. The heat continues to volatilize the tablets slowly and liberates gases therefrom, which gases are carbon solvents to a small degree. The solvent action loosens the carbon deposit in a very finely divided or powdered state and the powdered 90 carbon is discharged through the engine exhaust. While the de-carbonization starts almost immediately it continues to take 95

place slowly for one or two hours after the engine has been started up again and this gradual removal of the carbon avoids any chance of the carbon being broken up into 5 large particles which might lodge on the valve seats and clog the valves. Moreover the compound has the advantage that it can be put up into a handy commercial form, such as in tablets, and its use requires no 10 special training or skill.

What I claim as my invention is:—

1. A compound for use in removing carbon, comprising powdered zinc and a base therefor formed of wax.
- 15 2. A compound for use in removing car-

bon comprising a paraffin wax body or base and more than 30% of powdered zinc.

3. A compound for use in removing carbon, comprising powdered zinc, paraffin wax and stearin.

4. A compound for use in removing carbon, comprising the following ingredients in substantially the proportions given:

|                                          |     |    |
|------------------------------------------|-----|----|
| Powdered zinc -----                      | 60% | 25 |
| Paraffin wax -----                       | 25% |    |
| Stearin -----                            | 10% |    |
| Naphthalene (with coloring matter) ----- | 5%  |    |

In testimony whereof I affix my signature.

FRED R. REED.